

Aug. 7, 1934.

R. L. CHURCHILL

1,969,453

PACKAGING METHOD

Filed Jan. 16, 1933



Fig.1.



Fig.2.

Robert L. Churchill,  
Inventor:

By

Newton M. Garrison.

Daniel J. Mayne

Attorneys.

## UNITED STATES PATENT OFFICE

1,969,453

## PACKAGING METHOD

Robert L. Churchill, Kingsport, Tenn., assignor to  
Eastman Kodak Company, Rochester, N. Y., a  
corporation of New York

Application January 16, 1933, Serial No. 652,017

8 Claims. (Cl. 93—2)

This invention relates to the art of packaging and more particularly to a method whereby various types of wrappings produced from cellulose organic esters may be shrunk upon the article to be protected in such a manner as to produce a neat, tight wrap free from wrinkles.

When wrapping various articles of commerce such as bottles, cartons, packages of soap, metal containers and many other objects in cellulose acetate or other similar cellulose organic ester sheeting, it is often difficult, due to the peculiar physical properties of the material, to obtain a close, smooth fit without wrinkles. In other instances, especially when dealing with very thin sheeting, it is practically impossible to draw the material sufficiently tightly around the object to produce a smooth wrap without breaking. It has been proposed to obviate these difficulties by employing a type of sheeting which possesses self-shrinking properties. In such a case the sheet is merely wrapped around the article, sealed if desired, and permitted to shrink tightly thereover. One such type of sheeting is composed of cellulose acetate containing a substantial proportion, say 20-40% of a plasticizer such as diethyl phthalate, having a low boiling point and high vapor pressure, as compared to other plasticizers, which gives the sheeting markedly shrinking qualities.

It is the principal object of the present invention to improve upon the packaging art, especially with reference to the wrapping of various articles in thin cellulose organic ester sheeting. Another object is to provide a simple and effective method whereby a tight wrap free from wrinkles may be obtained. A specific object is to provide a method of tightening wrappers of cellulose acetate thin sheeting after they are applied to an article of commerce. Other objects will hereinafter appear.

I have found that these objects may be accomplished if the article, after wrapping, is subjected to the action of a solvent or swelling agent for the cellulose organic ester material employed and then permitted to dry. I have found that an even, uniform shrinkage takes place throughout the sheeting, which shrinkage has the effect of tightening the wrapper on the article and smoothing out wrinkles in a manner impossible when working by hand or even with the most perfect mechanical packaging equipment.

The method is extremely simple and may be carried out in a number of different ways. The article to be covered is first wrapped in cellulose acetate thin sheeting, for example, in the desired

manner, the edge portions in many cases being sealed by a suitable sealing agent or cement or simply by the application of heat and pressure. The wrapping material at this stage of the operation is relatively loose and has a tendency to wrinkle or buckle due to the uneven tension applied to the sheeting during application to the article, or in some cases, due to the particular form of the article itself. The wrapped article is next subjected to the action of a swelling agent or a solvent for the material of sheeting. This may be accomplished by moistening or wetting the outer surfaces of the wrapper with the agent by brushing or dipping. In some cases it may be desirable to apply the swelling or solvent agent in vapor form by suspending the wrapped article in a closed vessel containing the saturated vapor or by spraying the swelling or solvent agent thereon.

A typical example of the method according to the invention may be carried out as follows. An article, such as a cake of soap, a can of powder, a properly stoppered bottle of liquid or other article of commerce is suitably wrapped in a thin sheet of cellulose acetate, the edge portions of the wrapper being preferably sealed in any appropriate manner. A solution containing 67% denatured ethyl alcohol and 33% acetone is then prepared and the outer surface of the wrapper is moistened or wetted slightly by brushing the solution on with a soft brush. The wetted or moistened surface dries rapidly and most unexpectedly an almost immediate tightening or shrinking of the wrapper takes place, resulting in a smooth, neat package substantially free from wrinkles, buckled portions, or other unevenness.

The composition of the shrinking agent may vary widely. It must, however, be either a solvent or a swelling agent for the particular cellulose ester material dealt with. As a general rule, swelling agents are to be preferred due to their less drastic action on the sheeting. When using this latter type of agent less manipulative care is required in application than with an agent which has a pronounced solvent action. When working with relatively thick materials it may in some cases be necessary, either to employ a solvent alone, or a mixture of solvent and swelling agent. It will be apparent that the optimum proportions of solvent and swelling agent will necessarily be determined with reference to the type of material dealt with, its thickness, and other properties. In no case, however, will the agent be sufficiently drastic in its action to appreciably eat into or through the surface of the sheeting.

In the case of cellulose acetate sheeting, for

example, typical swelling agents which may be employed in accordance with the invention are methyl alcohol, ethyl alcohol, ethyl acetate, propyl acetate, and butyl acetate. Typical solvents include acetone, methyl acetate, diacetone alcohol, cyclohexanone, acetophenone and methoxy ethyl alcohol. If it is desired to reduce the evaporation rate of the agent, minor quantities of glycerin or similar polyhydric alcohols may be added.

As indicated above, application of the agent may be by simply brushing it onto the surface of the wrapper and permitting it to evaporate at room temperature. In some cases the wrapped article may even be dipped momentarily in a body of the liquid and then permitted to dry, or the article may be suspended for a short time in a closed space containing the saturated vapors of the liquid.

The two figures of the drawing graphically illustrate the effective tightening of a wrapper on an article of irregular shape, by means of my invention.

In Fig. 1 the numeral 1 indicates a properly stoppered bottle of liquid which has been relatively loosely wrapped in a thin, transparent sheet of cellulose acetate wrapping material (2) and sealed by means of solvent sealing agents or merely by application of heat and pressure. It will be noted that the material, even in spite of the most careful attention to wrapping, wrinkles and buckles and accordingly fits around the bottle somewhat loosely.

Fig. 2 illustrates the same package after the relatively loosely fitting wrapper has been treated by application of a shrinking agent such as described above. The wrapper (2) is now drawn tightly around the bottle and the wrinkles are completely smoothed out giving the package an extremely neat attractive appearance.

While I have described my invention with particular reference to cellulose acetate sheeting, it is equally applicable to methods of packaging involving the use of other types of single or mixed cellulose organic ester material, such as cellulose propionate, cellulose butyrate, cellulose stearate, cellulose acetate propionate, cellulose acetate butyrate and the like.

It will also be apparent that a wide latitude is permitted in the proportions of the various ingredients making up the shrinking bath or liquid. While I have described a bath containing approximately 67% of non-solvent (alcohol) to 33% of solvent (acetone), I may employ as much as 95% non-solvent, or more, with a correspondingly less amount of solvent, or even no solvent, if desired. The matter of proportions of any given combination of ingredients will also be governed largely by the particular type of sheeting dealt with.

The method of the present invention has many advantages over known methods of securing tightly fitting wrappings on package goods. Even the most efficient mechanical means of wrapping goods does not permit the sure and effective tightening of the wrapper made possible by the herein-described method. No complicated machinery or involved manipulative procedure is required, the method being particularly characterized by its extreme simplicity.

As many apparently widely different embodiments of this invention may be made without departing from the spirit and scope thereof, it is to be understood that I do not limit myself to the

specific embodiments thereof except as defined in the appended claims.

What I claim is:

1. The method of packaging which comprises enclosing an article in a wrapper comprising a non-self-shrinking sheet of cellulose organic ester material free from water-soluble compounds without tautening and subjecting the wrapper to the action of an organic swelling agent for the ester which upon evaporation tautens the wrapper. 80

2. The method of packaging which comprises enclosing an article in a wrapper comprising a non-self-shrinking sheet of cellulose organic ester material free from water soluble compounds without tautening and applying an organic swelling agent for the ester to the outer surface of the wrapper which upon evaporation tautens the material, and permitting the agent to evaporate therefrom. 90

3. The method of packing which comprises enclosing an article in a wrapper comprising a non-self-shrinking sheet of cellulose organic ester material free from water soluble compounds without tautening and applying to the outer surface of the wrapper, a solution comprising an organic swelling agent for the cellulose organic ester and a solvent for said ester therefor, and permitting the solution to evaporate, whereby the wrapper is uniformly shrunk and tautened 100 around the article. 105

4. The method of packaging which comprises enclosing an article in a wrapper comprising an organic sheet of cellulose acetate, applying to the outer surface of the wrapper an organic 110 swelling agent for the cellulose acetate, and permitting the agent to evaporate therefrom, whereby the cellulose acetate is uniformly shrunk and tautened around the article.

5. The method of packaging which comprises 115 enclosing an article in a wrapper comprising a sheet of cellulose acetate without tautening, applying to the outer surface of the wrapper an agent comprising 67% alcohol and 33% acetone, and permitting the agent to evaporate therefrom, 120 whereby the cellulose acetate is uniformly shrunk and tautened around the article. 120

6. The method of packaging which comprises enclosing an article in a wrapper comprising a non-self-shrinking sheet of cellulose organic ester 125 material free from water-soluble compounds, without tautening, and subjecting the wrapper to the action of a liquid which consists of a mixture of an organic non-solvent swelling agent for the cellulose organic ester and a solvent 130 therefor.

7. The method of packaging which comprises enclosing an article in a wrapper comprising a non-self-shrinking sheet of cellulose acetate free from water-soluble compounds, without tautening, and subjecting the wrapper to the action of a liquid which consists of a mixture of an organic non-solvent swelling agent for cellulose acetate and a solvent therefor. 135

8. The method of packaging which comprises 140 enclosing an article in a wrapper comprising a non-self-shrinking sheet of cellulose acetate free from water-soluble compounds, without tautening, and subjecting the wrapper to the action of a liquid which contains a major portion of an 145 organic non-solvent swelling agent for the cellulose acetate and a solvent therefor.

ROBERT L. CHURCHILL.